

May 24, 1949.

T. PRICE

2,470,790

MANUFACTURE OF ALLOYS

Filed April 24, 1945

Fig. 1.



Fig. 2.



Fig. 3.



Fig. 4.



Fig. 5.



INVENTOR  
TOMSON PRICE.

BY *John Newhouse*

ATTORNEY

## UNITED STATES PATENT OFFICE

2,470,790

## MANUFACTURE OF ALLOYS

Towson Price, Glen Ridge, N. J., assignor to Westinghouse Electric Corporation, East Pittsburgh, Pa., a corporation of Pennsylvania

Application April 24, 1945, Serial No. 590,046

2 Claims. (Cl. 75—176)

1

This invention relates to the manufacture of readily-oxidizable refractory metals of group VI of the periodic table of the elements, and more particularly molybdenum, tungsten and mixtures thereof, alloyed with metal such as chromium to protect the product against oxidation when heated.

The principal object of my invention, generally considered, is to provide alloys of molybdenum and/or tungsten containing sufficient chromium, whereby the readily-oxidizable refractory metal is protected when used at elevated temperatures in air or oxygen-containing atmospheres.

Another object of my invention is to provide chromium-molybdenum, chromium-tungsten and tertiary alloys, in which the chromium content is sufficiently high to prevent the other refractory metal or metals of group VI of the periodic table from oxidation at reasonably elevated temperatures, even though not enough to reduce the melting point of said other metal or metals more than a small amount.

A further object of my invention is to manufacture refractory alloys from metal of group VI of the periodic table, by making a balanced oxygen-carbon mixture of compounds of such metal in the metal proportions desired in the resulting product, heating in a protective atmosphere to drive off the resulting carbon monoxide, and sintering to coherent form, said oxygen-carbon mixture being initially treated either in a powdered or pressed form, and followed by a pressing, if necessary, to the shape desired prior to sintering.

A still further object of my invention is to manufacture molybdenum-chromium alloys by mixing, to obtain a balance between the oxygen and carbon atoms, chromium oxide, or carbide, with molybdenum oxide, and carbide or carbon, in proper proportions to produce the desired solid solution or alloy in the final product, heating the mixture in a reducing or protective atmosphere to effect a reaction or carbon reduction, with generation of carbon monoxide and the liberation of the free metal, grinding and/or sifting the reduced mass to remove coarse particles, removing if necessary any appreciable residual carbon, pressing into slugs, and sintering to coherent form.

Other objects and advantages of the invention will become apparent as the description proceeds.

Referring to the drawing:

Fig. 1 is a vertical sectional view of a receptacle for mixing the selected materials to produce a

balanced oxygen-carbon mixture of compounds of the selected metal.

Fig. 2 shows the apparatus of Fig. 1 during a subsequent stage in which the mixture is being dried, as by means of steam, while stirring.

Fig. 3 is a vertical longitudinal sectional view of an electrical reducing furnace in which the mixture is first heat-treated.

Fig. 4 is a vertical sectional view of a hydraulic press in which slugs of the mixture, reduced in the furnace of Fig. 3, are formed.

Fig. 5 is a vertical sectional view of a sintering furnace in which the slugs produced in the press of Fig. 4 are finally treated.

Difficulty is experienced in the manufacture of alloys, such as those adapted to resist oxidation at elevated temperatures, and involving a combination of a refractory metal, such as molybdenum, the oxide of which is readily reducible by hydrogen, and a metal such as chromium, the oxide of which is not readily reducible by hydrogen. Chromium is rather oxidized by hydrogen containing water vapor. If a mixture of the oxides of the two metals is heated in hydrogen, the molybdenum oxide is reduced leaving the chromium oxide mixed with the metallic molybdenum. In order to get chromium to alloy with molybdenum, the molybdenum has to be sintered at high temperature in hydrogen to effect some dissociation of the chromium oxide and absorption of the chromium so formed by the molybdenum.

The efficient way to reduce chromic oxide to chromium is by carbon. However, if carbon is used to reduce molybdenum oxide, the result is molybdenum carbide or a considerable impregnation of molybdenum with carbon which is difficult to eliminate.

I will now describe the preparation of a molybdenum-chromium alloy in proportions such that the melting point will be near that of molybdenum, that is, above about 90% of the melting point of molybdenum measured in degrees C. It will, however, be understood that a similar process is applicable to the manufacture of other metal alloys of group VI of the periodic table, whether alloys of molybdenum and chromium or not. That is, my process includes the manufacture of alloys of tungsten and chromium; and tungsten, molybdenum and chromium as well as molybdenum and chromium.

Referring to the drawing in detail, there is shown in Fig. 1 a receptacle 11 in which is placed a desired quantity 12 of a mixture of powdered oxide of chromium and powdered carbide of

molybdenum. The chromium oxide may be chromic oxide,  $\text{Cr}_2\text{O}_3$ , or other oxide of that metal, and the molybdenum carbide is that represented by the formula  $\text{MoC}$ . As an alternative, however, I may substitute chromium carbide for the oxide, or use no carbide, rather substituting an equivalent mixture of oxide and finely-divided carbon, such as lamp black or powdered coal, but the purer the better.

Upon this mixture is poured molybdenum oxide, such as the trioxide or dioxide, mixed with or suspended in water. During the addition of the suspension 13, the mixture is constantly stirred, as by means of a rod 14, while the receptacle is heated, preferably by means of steam 15. On account of drying with constant stirring, segregation of the liquid is avoided and a mixture of oxides and carbides, or oxides and carbon, uniformly commingled together is obtained. As a further alternative, I may introduce the chromium as a water-soluble salt, such as chromous acetate, dissolved in water and mixed with the oxide and carbide of molybdenum, or said oxide and finely-divided carbon, to get not only the desired oxygen-carbon balance but also the desired metals ratio.

I may add a small proportion, that is from about .01% to about 1%, as a preferred range, of one or more of metals of the nickel-cobalt-iron group, that is, one of series 4, group VIII of the periodic table as in the form of a soluble salt or salts, along with the chromium salt, to increase the facility with which the molybdenum or tungsten and the chromium combine, thereby decreasing the necessary sintering temperature of the alloy and giving it a denser grain structure so that it is more readily protected against oxidation.

The mixture above described, which may be in accordance with the left hand side of the following equation, when heat-treated to effect a reaction between the components, theoretically gives an alloy of about 91% molybdenum and 9% chromium:



To effect a reaction in accordance with the above formula, the dry well-mixed mass is then placed in suitable receptacles or boats 16, and passed through a reducing furnace 17. Such a furnace may comprise a suitably-insulated tube 18 of refractory material such as alumina, surrounded by a coil 19 of molybdenum or tungsten through which electricity is passed to supply the heating power. The atmosphere in the furnace may be protective or reducing. It is desirably dry hydrogen, that is hydrogen preferably having a dew point of not higher than  $-60^\circ\text{C}$ , although other dry atmospheres may be used. If desired, the furnace may be of the type illustrated in Fig. 1 of the Hall et al., application, Ser. No. 579,080, filed February 21, 1945, now Patent No. 2,431,690, dated December 2, 1947, and owned by the assignee of the present application.

During this treatment the furnace need only be operated at a relatively low temperature, but it must be one high enough to effect a reaction between the oxide and carbide, or a reduction of the oxide by the finely-divided carbon. Such temperatures are between about  $800^\circ$  and  $1000^\circ\text{C}$ , although higher temperatures may be employed if obtained gradually so as not to appreciably sublime the molybdenum trioxide, if used, before reduction. The length of treatment may be from one to two hours or longer. Atmospheres other

than hydrogen may be used and produced by mixing with nitrogen a small proportion of hydrogen, carbon monoxide or other reducing gas. The atmosphere is modified during the treatment by the evolution of carbon monoxide, in accordance with the above equation.

After the reaction has been effected, the product is removed from the furnace and either sifted to remove lumps or ground and sifted so that it is in the form of powder of fine particle size. If it contains an undesirable excess of carbon or carbide, this may be removed by mixing with a sufficient amount of molybdenum oxide to provide the necessary oxygen for removing the carbide as carbon monoxide upon subsequent heating. A slight excess of the oxide is not objectionable as it either reduces or vaporizes during the subsequent heat-treating process.

The powdered metal or mixture is then pressed into slugs or articles 21 of form desired, as in a die 22 by means of a plunger 23 operated by a hydraulic press 24, so that sufficient coherence of the particles is provided to allow for necessary handling of the formed slugs.

The pressed slugs or other articles 21, after removal from the die, are placed in a sintering furnace 25 which may be the same or like the furnace 17, except that said slugs are there treated in dry hydrogen, hydrogen-bearing gas, or a protective gas such as argon, helium or nitrogen. Hydrogen is desirably used if it is desired to eliminate residual carbon from the slugs, as it combines therewith to produce hydrocarbons which pass off with the flowing gas. However, if the slugs produced are free from carbon, one of the other gases mentioned may be employed. The temperatures of treatment are in accordance with conventional practice in sintering such metal, the preferred temperature depending on whether it is mainly molybdenum or tungsten. As an alternative, the slugs may be sintered in accordance with the sintering treatment for such chromium alloys, described in the Ramage application, Ser. No. 559,693, filed October 21, 1944, and owned by the assignee of the present application.

Instead of the foregoing, I may use the following equation which would theoretically yield an alloy of about 9.8% chromium:



From the foregoing equations and explanation, it will be seen that the expression "balanced oxygen-carbon mixture," as used in this application, means that the mixture which is prepared has, prior to firing, the proper ratio between the ingredients, so that after the reaction product, carbon monoxide, has been driven off, only metal remains which is free, or substantially free, from both carbon and oxygen.

As an alternative, a balanced carbide and oxide mixture could be pressed into a slug and slowly heated, as in the furnace of Fig. 5, in a hydrogen or other protective atmosphere, to first drive off the carbon monoxide produced during the reaction, and then sinter the resulting metal particles to form a coherent alloy.

Although the foregoing equations have been shown using molybdenum trioxide, other oxides of molybdenum or mixtures thereof could be substituted and the process is suitable for the production of other alloys or mixtures of refractory metals of group VI of the periodic table.

One of the big advantages of this method of alloy formation is that the ingredients can be

prepared in a pure form and mixed in the molecular proportion required to give the product desired, the carbide or carbon protecting material such as chromium, which is oxidizable by water vapor, and the oxide of which is not ordinarily reducible by hydrogen.

Although preferred embodiments of my invention have been disclosed, it will be understood that modifications may be made within the spirit and scope of the appended claims.

I claim:

1. The method of manufacturing coherent chromium alloys of metals selected from the group consisting of molybdenum and tungsten, comprising making a mixture of a powdered oxide and a powdered carbide of the selected metal and a solution of a chromium compound in an amount sufficient to yield approximately 9% of chromium in the product and containing from about .01% to about 1% of at least one metal of series 4, group VIII, of the periodic table, in the form of a soluble salt, to facilitate combination of the chromium with the selected alloying metal, the proportions of the ingredients and the ratio between the carbide and the other ingredients being such that after the reaction product, carbon monoxide has been driven off during the operation of the method, the metal produced is sub-

stantially free from both carbon and oxygen, constantly stirring the mixture and heating to a temperature of about 100° C., thereby avoiding segregation of the liquid and obtaining a uniformly commingled dry mixture, loading said well-mixed mass in suitable receptacles, and heating said loaded receptacles slowly in an atmosphere of dry hydrogen to a temperature between about 800° and 1000° C., continuing said treatment for from one to two hours, and cooling the reduced material.

2. The method as defined in claim 1, in which the chromium compound is the acetate.

TOWSON PRICE.

#### REFERENCES CITED

The following references are of record in the file of this patent:

#### UNITED STATES PATENTS

| 20 | Number    | Name                  | Date          |
|----|-----------|-----------------------|---------------|
|    | 1,308,907 | Keyes -----           | July 8, 1919  |
|    | 1,418,081 | Laise -----           | May 30, 1922  |
|    | 1,665,636 | Marden et al. -----   | Apr. 10, 1928 |
| 25 | 1,731,267 | Rich -----            | Oct. 15, 1929 |
|    | 2,205,386 | Balke -----           | June 25, 1940 |
|    | 2,242,759 | Schlecht et al. ----- | May 20, 1941  |